

No. 709,488.

Patented Sept. 23, 1902.

W. S. HUNTINGTON.  
PROCESS OF MAKING ARTIFICIAL LUMBER.

(Application filed Feb. 18, 1901.)

(No Model.)

Fig.1



Fig. 2



Fig. 3



Witnesses:

Raphael P. Potts  
Richard Kloman

William S. Huntington, Inventor  
by Ken Page & Coopers Atlys

# UNITED STATES PATENT OFFICE.

WILLIAM S. HUNTINGTON, OF NEW YORK, N. Y., ASSIGNOR TO THE COMPOSITE BOARD COMPANY, A CORPORATION OF NEW YORK.

## PROCESS OF MAKING ARTIFICIAL LUMBER.

SPECIFICATION forming part of Letters Patent No. 709,488, dated September 23, 1902.

Application filed February 18, 1901. Serial No. 47,709. (No specimens.)

*To all whom it may concern:*

Be it known that I, WILLIAM S. HUNTINGTON, a citizen of the United States, residing in the borough of Manhattan, in the city and State of New York, have discovered a new and useful Process of Making Artificial Lumber, of which the following is a specification, reference being had to the drawings accompanying and forming a part of the same.

10 The invention or discovery which forms the subject of my present application for Letters Patent is the result of an extended series of experiments conducted with the object of producing from wood-pulp a substitute for the finer grades of wood used in cabinet-making, the finish of cars, ships, and the like and in which lightness, strength, and durability, with a certain degree of flexibility, are of equal importance with the capability of taking a high finish.

So far as I am aware no wood-pulp product, either in a substantially pure state or combined with the usual fillers, has heretofore been produced in a condition to meet the practical requirements of such uses as those to which hard-wood veneers and the like are generally applied, mainly because of the impossibility of obtaining by any known process slabs or sheets of compacted pulp possessing a sufficient degree of hardness coupled with flexibility; but this objection I have succeeded in overcoming by a process of manufacture which yields slabs, sheets, or boards or in general an artificial lumber having the general appearance and the more desirable characteristics of natural wood, but of lighter weight and greater flexibility than the latter and free from all tendency to crack, split, check, or splinter and capable of withstand-  
40 ing the action of moisture and effects of heat without blistering.

In carrying out my invention the main object is to impregnate the body of the compacted wood-pulp with a material or compound which will impart to the body hardness and flexibility without impairing the tenacity which is due to the natural matting or felting properties of the fibers, and in order to secure this result I have found it necessary to depart from the usual processes followed in the manufacture of papersheets and

boards in several particulars, as will herein-after more fully appear.

In order that the invention in such detail as will enable a person skilled in the art to practice it may be fully understood, I shall describe the process which I have adopted as the best now known to me.

It will be understood that a proper wood is first ground in any of the usual ways and the desired quantity put in a beater-engine, together with a certain proportion of "sulfite," as the long-fibered pulp digested with bisulfite liquor is known in the market, together with the usual quantity of alum and size. The proportion of sulfite may vary; but it is somewhat less than is ordinarily used in the manufacture of the better grades of paper. I also introduce into the beater-engine such materials as will have a tendency to impart to the finished product solidity and hardness and, to the extent to which they remain, greater tenacity. The substances best suited for this purpose I have found to be litharge, ground white lead, and casein. A rigid observance of proportions is not necessary; but good results will be found to follow the employment with five hundred pounds of ground wood of about forty pounds of sulfite, eight pounds of size, twelve pounds of ground white lead, ten pounds of litharge, and twenty pounds of alum, the latter being first dissolved in hot water. About twelve pounds of casein, which is also to be mixed in hot water, should be added after the other ingredients named have been combined. This admixture is thoroughly beaten in the engine and then run or pumped off into a storage-tank, in which it is allowed to stand generally for about thirty minutes or until a scum forms on the surface. This latter being removed, the mixture is transferred to the vats of an ordinary cylinder-machine. Two or more cylinders are used to pick up the pulp by suction and deliver it in thin layers or films on an endless felt belt, which in turn deposits the film onto a press-roll, on which the film or films are wound until the accumulated convolutions give the desired thickness of material. The latter is compacted by the press-roll, then cut transversely, and deposited by suitable means onto a carriage. The wet

slabs or sheets are then hung in a drying-chamber or kiln, which should be constructed with special reference to the prevention therein of any pronounced circulation of air, in 5 this respect differing from that class of drying-rooms or kilns in which steam-pipes are placed overhead and the hot air forced downward by means of fans or the like. For this purpose it is merely necessary to have a compartment which can be tightly closed and to 10 arrange the steam-pipes near the floor.

If the wet slabs or sheets produced as above described be dried without further treatment, they will not be suitable for the uses contemplated herein, mainly because of their brittleness; but by drying them in the presence of the vapor or fumes of a material which is capable of imparting hardness and flexibility to them they appear to become impregnated with such material and to acquire these properties to a marked degree. This result may be secured to varying extents and by the use of various hardening compounds; but I prefer to use as the materials for producing the 25 said vapor or fumes litharge, bicarbonate of soda, casein, and sulfuric acid and the flour or dust of wood, applying the same in the following manner: I provide for use in the kiln any suitable receptacles, which are to be 30 placed on the heating-pipes. In the bottom of each I place about six pounds of litharge, over which I deposit a layer of four pounds of casein. Over this I sprinkle about one pound of bicarbonate of soda and cover the 35 whole with a layer about two inches thick of wood-dust from the sanding-machines, saturated with sulfuric acid. I then pour over the whole sufficient sulfuric acid to entirely decompose the other ingredients. The acid 40 filtering down through the dust or flour of wood attacks the materials beneath, developing fumes, which fill the chamber and act upon the drying slabs or sheets, imparting thereto the peculiar hardness and flexibility 45 which characterizes the product which I manufacture. The drying process is conducted, as above stated, in a closed or sealed chamber and at a temperature of about 120°, which is maintained for about twenty-four hours. 50 At the end of this period the dried and hardened sheets are removed and after having been trimmed or edged are sprinkled with water at points where warping or bulging has occurred and then placed under a hydraulic 55 press and subjected to pressure to restore them to their original flat condition. The sheets are then passed between hot calendering-rolls to surface and thoroughly free them from moisture, after which they are sanded 60 to give them a true surface and to reduce them to the desired thickness. In this condition the sheets are useful for many purposes; but to secure the full benefit of my improvement I apply to the smoothed surfaces of two, three, 65 or more sheets a suitable glue, such as that now commercially known as "casein-glue," and unite them under pressure into compos-

ite boards or sections of any desired thickness. By the same operation I impart to the boards such forms as they are required to 70 have in use, as head-linings for cars or the like. After this treatment and when the glue is dried and the body of the material has acquired a permanent shape or set the material is treated in the same manner as wood or veneers with fillers, varnish, or paint of any desired kind. 75

In carrying out the above-described process I may employ any suitable apparatus or mechanism, the invention, broadly considered, not being limited to the use of any precise form. For purpose of illustration, however, I have shown a simple form of apparatus which is capable of being used for the purpose, omitting the calendering-rolls and 85 presses, as these are such well-known devices as to require no special description.

Figure 1 is a view, partly in side elevation and partly in section, of the apparatus for forming the sheets or slabs. Fig. 2 is a view 90 of the drying-chamber or kiln, a portion of the side wall being removed to show the interior arrangement. Fig. 3 is a perspective view of one of the finished boards or sections of material. 95

A B indicate a pair of pulp-vats, within which are mounted the screen-cylinders C, preferably having communication with a suitable suction apparatus, as is usual in such cases. 100

D is an endless belt of felt, which is pressed against the cylinders C by couch-rolls E to receive the layers or films of pulp taken up by the cylinders. The belt D leads to the drum or press-roll F, which receives and winds 105 up the film until the desired thickness is obtained. Coöperating with the drum F is a wringer-roll G in adjustable bearings, which is used to express the surplus from and to compact the layers wound on the drum. 110

H is a chamber capable of being tightly closed and containing a series of steam-pipes K near the floor of the same.

L designates some of the slabs or sheets as taken from drum F and shown as hung in the 115 chamber H.

M M are the receptacles containing the hardening materials above described and placed on the pipes, so as to be heated thereby.

In Fig. 3 the slab L is shown bent to its 120 final form.

From the above description of the invention it will be seen that the presence throughout the body of felted or matted fibers of material, which impart to the compacted mass hardness and flexibility, is essential. 125

Some of the necessary ingredients, as explained, are incorporated with the pulp; but so much of these is removed in the beater-engine and vats by the washing action which 130 the pulp undergoes until it is lifted out of the vats by the cylinders that resort must be had to special means for impregnating or treating the substance to impart to it the desired prop-

erties. The most effective method of accomplishing this is that described, and which consists in drying the sheets by heat in the presence of the vapor or fumes of the hardening materials. I have, however, found that similar results may be secured by other means, which in a broad sense I regard as the equivalent to that described. For example, I have mixed together the materials used in the receptacle in the drying-chamber and subjected them to a low heat in a closed receiver until the decomposition has taken place. This leaves a quantity of liquid, together with some sediment. If the liquid be drained off and mixed with the pulp in the vats, the sheets formed from such pulp after being dried in a closed chamber without further treatment will be found to produce to a degree the hardness and flexibility characteristic of the product of the preferred process. It will be seen, therefore, that the order of the steps of the process in its broader aspects, and particularly in so far as the incorporation of the hardening material is concerned, is not material.

25 What I claim as my invention is—

1. The process of making artificial lumber which consists in forming and compacting wood-pulp into moist slabs or sheets, and drying the same in a heated atmosphere charged 30 with materials capable of hardening and imparting flexibility to the same.

2. The process of making artificial lumber, which consists in forming and compacting wood-pulp into slabs or sheets, drying the same by heat in the vapor or fumes of materials capable of imparting hardness and flexibility to the same, and then flattening and finishing the sheets, as set forth.

3. The process of making artificial lumber 35 which consists in subjecting slabs or sheets

of wood-pulp in a wet state to the action of heat in the presence of the vapor or fumes of materials capable of imparting hardness and flexibility to the slabs and then superposing and uniting the dry slabs by pressure, as set 45 forth.

4. The process of making artificial lumber which consists in subjecting individual wet slabs or sheets of wood-pulp to the action of heat in the presence of materials capable 50 of imparting hardness and flexibility to the same, then subjecting the slabs to pressure to correct the distortion incident to drying, then applying adhesive material to the slabs and superposing and uniting two or more of 55 the same by pressure, as set forth.

5. The process of making artificial lumber, which consists in drying individual wet slabs or sheets of wood-pulp in an atmosphere charged with materials capable of imparting 60 hardness and flexibility thereto, then subjecting the slabs to pressure to correct the distortion incident to drying, then resurfacing the slabs to impart a smooth surface thereto, then applying an adhesive material to 65 the surfaces, and then superposing and uniting two or more of the slabs and simultaneously imparting the desired form to the finished product by means of pressure, as set forth. 70

6. The process of making artificial lumber which consists in drying wet slabs or sheets of wood-pulp by the action of heat in the vapor or fumes produced by sulfuric acid, litharge, casein and an alkali, as set forth.

WILLIAM S. HUNTINGTON.

Witnesses:

JOHN C. KERR,  
RICHARD DONOVAN.